

June 2, 1953

E. C. BERTOLET, JR

2,640,795

FRICITION ELEMENT AND METHOD OF FORMING SAME

Filed Aug. 14, 1951

*Fig. 1*



*Fig. 2*



*Fig. 3*



*Fig. 4*



*Fig. 5*



*Inventor*

*Elmer C. Bertolet Jr.*

*by: Gary Desmond + Parker*

*Attnys.*

## UNITED STATES PATENT OFFICE

2,640,795

FRICITION ELEMENT AND METHOD OF  
FORMING SAME

Elmer C. Bertolet, Jr., Lititz, Pa., assignor to  
Raybestos-Manhattan, Inc., Passaic, N. J., a  
corporation of New Jersey

Application August 14, 1951, Serial No. 241,855

7 Claims. (Cl. 154—81)

1

This invention relates to improvements in the production of friction elements and particularly friction rings of the endless type suitable for use as automobile clutch facings, generally formed of strips of material wound in spiral fashion to form a coiled annulus.

More particularly, the present invention is directed to the production of clutch facings wherein a strip comprised of asbestos, heat-hardenable binder, and friction augmenting agents is shaped or folded longitudinally to impart to it an arcuate, V-shape, or other deformed cross-section, prior to or while simultaneously coiling it spirally to form an annulus, with internesting of adjacent coils. This results in a structure, after densification and cure of the binder, which is devoid of any incipient or potential planes of cleavage which may extend directly from one face of the facing to the opposite face thereof, and thus has high resistance to tear or rupture of the facing when used in conjunction with engines which develop high rotative speeds, as described, for example, in United States Patent No. 2,096,692 to O. H. Cilley, where employment of woven asbestos fiber is indicated.

It is an object of the present invention to form friction elements of the foregoing class of novel composition and in an economical manner by elimination of the requirement and likewise the expense of spinning, twisting, winding and weaving entailed in the production of woven materials.

The present invention also makes possible the production of products of greater uniformity due to ability to control thickness of the base and of the coatings applied thereto, and of end products of more uniform weight from windings of the same lengths of treated strip material.

Thus, in accordance with the present invention, I employ strips cut from webs or sheets of carded asbestos fibers of specific formation and in a novel manner as will hereinafter be more particularly described.

The asbestos sheet material which I employ is in general produced by carding and dry felting asbestos fibers of spinning grade lengths from a mix which usually contains a percentage of cellulose fibers to act as a carrier in the carding operation. For use in friction materials of the class herein contemplated, the cellulose fibers in the mix should be from 10% to 45% by weight of the total of the foregoing two kinds of fibers. Examples of suitable cellulose fibers are cotton, rayon, flax, jute, hemp, or the like. Although such cellulose fibers have a tendency to carbonize on the operative surface of the friction ele-

2

ment under the frictional heat encountered, such surface carbon formation has been found to be a desirable friction modifying agent, particularly for the purpose of minimizing the undesirable tendency of "fading" under the frictional heat of operation, as is the case when cellulose fibers are omitted.

Further objects and advantages of the present invention and the details of construction thereof will be explained in connection with the following specification and accompanying diagrammatic drawings, wherein:

Fig. 1 is a plan view, with parts broken away, of a sheet of carded and condensed web of fibrous asbestos sheet material impregnated with a friction material composition cement, in accordance with the present invention.

Fig. 2 is a perspective view of a strip cut from the impregnated sheet of Fig. 1, and folded longitudinally prior to winding.

Fig. 3 is a section of a clutch facing winding having an inverted V-shaped formation, before compression and cure, and

Fig. 4 is a similar view after compression and cure.

Fig. 5 is a view of the face of the clutch facing after compression and cure.

Referring to the drawings, the reference numeral 10 indicates a web or sheet of carded and condensed asbestos material, composed of the mixture of fibers previously indicated. The asbestos fibers are of long or spinning grade length such as from  $\frac{1}{8}$  to 1 inch, and predominantly of a length greater than  $\frac{1}{2}$  inch, as distinguished from the shorter length fibers generally employed in making asbestos paper in aqueous slurries. The mixture of fibers is carded in a manner well known to the art through use of carding machines to form relatively thin webs with the fibers substantially uniformly distributed and lying in a predominantly directionalized, oriented and parallelized formation, having individual thicknesses of from about .003 to .009 inch before application of pressure. If desired a plurality of these webs may be superimposed to build up the desired ultimate weight or thickness of the desired sheet, and in the practice of the present invention a laminate of two or more plies is generally employed.

Two or more webs are preferably laid up together and then jointly subjected to a sizing operation wherein the material is totally immersed in a dilute solution of a sizing or bonding material, and condensed by means of rolls so as to consolidate the web and to effect a uniform dis-

tribution of said sizing or bonding material, and then dried. Such composites are relatively free from holes, lumps and other unevenness due to the leveling effect of multiple layers.

The sizing operation comprises the incorporation of conventional sizing, bonding or adhesive materials such as starches, latex, glues, shellac, aqueous solutions or dispersions of resinous materials such as urea, melamine or phenol formaldehyde resins, and the like, in the web to additionally strengthen the composite carded structure and to set it in its densified condition. The sizing operation is preferably so controlled as to incorporate from about one to about two per cent of solids in the web by weight thereof, and to thereby leave the web in a condition of porosity such that it can subsequently be readily impregnated with saturants. For example, the foregoing web material is of such porosity and absorbency that it can absorb three to four times the weight of impregnant that can be incorporated under like circumstances in a water-laid paper of comparable thickness. On the other hand the present consolidated web does not have the undue absorbency of a "lofted" or unsized web, and thereby permits employment of relatively low ratios of solvent to binder. In addition to the undesirable properties of "lofted" carded webs such as poor tensile strength, bulk, requirement for support and poor drying qualities, lofted webs require very high proportions of solvent to binder solids for proper saturation and incorporation of equal amounts of solids.

In addition to the economies of the foregoing carded and condensed asbestos web material over woven asbestos textiles, this web material is capable of production in finished thickness below that of conventional woven asbestos textiles and in a much more uniform condition, and can be more thoroughly and more uniformly impregnated. As previously indicated the same applies in general to water-laid fibrous asbestos papers, which have the added deficiency of low tensile strength and lack of deformability and distortability, as distinguished from the high tensile strength of the web material herein employed, particularly in the direction of its fiber orientation, and its ability to appreciably stretch and be deformed without rupture which is of particular advantage for the purpose of the present invention as will herein-after appear.

As one example of the material found suitable in the practice of the present invention, a mixture of 75% by weight of spinning grade asbestos and 25% by weight of cotton was carded and three plies laid together. This was then impregnated with a starch solution to incorporate 2% by weight of the starch, consolidated by rolling and dried, to form a sheet having a thickness of approximately .012 inch.

Before cutting the sheet 10 into strips and shaping, it is impregnated with a cement comprised of heat-hardenable organic binder and friction material fillers 11, conventionally employed in friction material compositions. Such compositions in general comprise inorganic fillers such as litharge and barytes, and heat-hardenable binders, such as drying oils, thermo-setting synthetic resins, rubbers, and the like, generally, although not necessarily, as a mixture of two or more of such binders. The resins are generally of the phenolic type, such as the phenol aldehydes, particularly phenol formaldehyde, which may be of an oil modified type. The rubber may be either natural rubber or a synthetic rubber such

as polychloroprene, butadiene-styrene copolymer, or the like, and such rubbers may be in modifying combination with the resins or in admixture. These solids are formed into a cement with from about one part of hydrocarbon solvent for the soluble components to one part of total original solids. The composition further includes vulcanizing agents for the rubbers. A typical example of such binder composition, for the purpose of illustration and not limitation is as follows, the proportions given being in parts by weight:

|                   |        |
|-------------------|--------|
| Rubber            | 7.40   |
| Accelerator       | .22    |
| 15 Sulphur        | 7.92   |
| Barytes           | 31.90  |
| Litharge          | 24.90  |
| Graphite          | 1.62   |
| Rosin             | 1.08   |
| 20 Phenolic resin | 25.06  |
|                   | 100.10 |

The web material is preferably impregnated and 25 saturated by passing it through the cement solution and excess removed by suitable means, such as squeeze rolls, and then dried to remove the solvent but without cure of the binder. The total amount of the binder solids is approximately 30 equal to the weight of the fibrous materials, or from about 40 to about 60% by weight of the composite.

The impregnated sheet material is then cut 35 into strips of for example one-half inch in width, with the oriented fibers running generally longitudinally of the strip, and then longitudinally, shaped or deformed, to for example the strip 12 of Fig. 2 having an inverted V-shape cross-section. This shaped strip is thereafter helically wound 40 with adjacent coils in internesting relationship to form the annulus of Fig. 3 by suitable means and in the manner indicated in the aforesaid patent. Due to the elastic nature of the web base, its high tensile strength and directionalized fiber 45 formation it may be conveniently stretched without rupture in the shaping and winding operations and has adequate elasticity or stretchability required for elongation of the shaped strip at the apex of the V, and for ready contraction at the 50 edges of the strip when wound as shown in Fig. 3, or conversely if it were to be wound with the apex of the V inwardly, or any other desired symmetrical cross-section.

The coiled annulus is therefore subjected to 55 heat and pressure by suitable means, such as, for example, in a mold to densify it, and cause the binder to flow to permeate and consolidate the windings, and to heat-harden or cure the binder content, after which the unit is subjected to a 60 finishing operation, such as by surface grinding. The rivet holes 13 may be formed during the molding operation or formed subsequently by drilling and counter-boring.

It will be understood that although I have 65 in the foregoing described the preferred embodiment of my invention, as non-fully equivalent alternative, I may employ flat wound coils of the same tape or strip composition, since even in such case the economy of the carded asbestos web material over woven textiles is inherent, and its employment has the advantage of ability to control desired thickness of base material and amount of impregnant, and greater uniformity of surface and thickness than water-laid asbestos 70 papers or woven asbestos textiles, and the ability

to be better and more uniformly saturated with impregnants than such materials.

I claim as my invention:

1. An endless clutch facing comprised of a spirally wound strip of thin, flexible, consolidated and condensed carded long fiber asbestos web material of relatively high porosity, the fibers extending generally longitudinally of the strip, said strip being longitudinally folded to provide a symmetrical cross-sectional form and the coils thereof being secured together in internesting relationship.

2. An endless clutch facing comprised of a spirally wound strip of thin, flexible, consolidated and condensed carded long fiber asbestos web material of relatively high porosity including cellulose fibers in the proportion of from 10% to 45% by weight of said fibers, the fibers extending generally longitudinally of the strip, said strip being longitudinally folded to provide a symmetrical cross-sectional form and the coils thereof being secured together in internesting relationship.

3. A friction element suitable for use as a clutch facing, comprising an annular body formed of a convoluted strip of consolidated and condensed carded asbestos fibers of spinning grade length including cellulose fibers in the proportion of from 10% to 45% by weight of said fibers, said strip being of relatively high porosity and the fibers thereof being generally oriented in a direction longitudinally of said strip, said strip including heat-hardenable binder, said element being compressed to consolidate the convolutions upon each other and heat treated to harden the binder.

4. A friction element suitable for use as a clutch facing, comprising an annular body formed of a convoluted strip of consolidated and condensed carded asbestos fibers of spinning grade length including cellulose fibers in the proportion of from 10% to 45% by weight of said fibers, said strip being of relatively high porosity and the fibers thereof being generally oriented in a direction longitudinally of said strip, said strip being impregnated with a heat-hardenable binder-friction material filler composition cement, said element being compressed to consolidate the convolutions upon each other and heat treated to harden the binder.

5. A friction element suitable for use as a clutch facing, comprising an annular body formed of a convoluted strip of consolidated and condensed carded asbestos fibers of spinning grade length and including cellulose fibers in the proportion of from 10% to 45% by weight of said fibers, the fibers of said strip being generally oriented in a direction longitudinally thereof.

said strip being of a relatively high porosity and impregnated throughout its thickness with a heat-hardenable binder-friction material filler composition cement, said strip being further longitudinally folded to provide a symmetrical cross-sectional form and the convolutions thereof being in internesting relationship, said element being compressed to consolidate the convolutions upon each other and heat treated to harden the binder.

6. The method of forming a friction element suitable for use as a clutch facing, which comprises impregnating a strip of relatively thin, porous, flexible asbestos sheet material composed of carded and condensed spinning grade asbestos fibers substantially uniformly distributed and directionalized longitudinally of the strip, with a heat-hardenable binder-friction material filler composition cement, drying solvent content from said cement, convolutely winding said strip material to form an annular body, and subjecting said body to heat and pressure to consolidate said strip.

25 7. The method of forming a friction element suitable for use as a clutch facing, which comprises cutting a sheet of relatively thin, porous, flexible asbestos sheet material composed of carded and condensed spinning grade asbestos fibers including cellulose fibers in the proportion of from 10% to 45% by weight of said fibers wherein the fibers are substantially uniformly distributed and lie in a predominantly oriented and parallelized formation, into strips wherein the fibers extend generally longitudinally of the strip, impregnating said strip throughout its thickness with a heat-hardenable binder-friction material filler composition cement, drying solvent content from said cement, folding said strip longitudinally to provide it with a symmetrical cross-sectional form, convolutely winding said strip material to form an annular body, and subjecting said body to heat and pressure to consolidate the convolutions upon each other and to harden the binder.

ELMER G. BEETOLET, JR.

References Cited in the file of this patent  
UNITED STATES PATENTS

| Number        | Name             | Date          |
|---------------|------------------|---------------|
| 50. 1,420,883 | Stanley -----    | June 27, 1922 |
| 1,437,438     | Nanfeldt -----   | Dec. 5, 1922  |
| 1,465,389     | Fisher -----     | Aug. 21, 1923 |
| 1,771,749     | Eisenhardt ----- | July 29, 1930 |
| 2,096,692     | Cilley -----     | Oct. 19, 1937 |
| 55. 2,218,535 | Judd -----       | Oct. 22, 1940 |
| 2,264,901     | Gosling -----    | Dec. 2, 1941  |
| 2,546,056     | Batchelor -----  | Mar. 20, 1951 |